

(No Model.)

C. E. BILLINGS.

COMMUTATOR BAR FOR DYNAMO ELECTRIC MACHINES.

No. 392,490.

Patented Nov. 6, 1888.

Fig. 1



Fig. 2



Fig. 3



Witnesses:

W. M. Yorkman  
Lewis L. Richards.

Inventor:  
Charles E. Billings,  
By Willard Eddy,  
Atty.

# UNITED STATES PATENT OFFICE.

CHARLES E. BILLINGS, OF HARTFORD, CONNECTICUT.

## COMMUTATOR-BAR FOR DYNAMO-ELECTRIC MACHINES.

SPECIFICATION forming part of Letters Patent No. 392,490, dated November 6, 1888.

Application filed December 4, 1886. Serial No. 220,676. (No model.)

*To all whom it may concern:*

Be it known that I, CHARLES E. BILLINGS, of Hartford, Connecticut, have invented a new and useful Commutator-Bar for Dynamo-Electric Machines, which is described in the following specification and is illustrated by the accompanying drawings.

This invention relates to commutators of dynamo-electric machines, whether motors or generators; and it consists of a commutator-bar, a commutator-strip, or a "segment" of the commutator, variously so called, which is formed of a single piece of pure copper and has two arms whose longitudinal axes form an angle with each other.

15 Commutator-bars have heretofore been made of a single piece of brass, bronze, or other electrically-conductive alloy cast in the described form, but on account of the difficulty of casting pure copper have not been made of a single piece of that metal in the specified form. Commutator-bars have also been made in two arms separately constructed, and soldered, screwed, or otherwise joined together. According to this method the main arm of the commutator-bar has sometimes been formed of pure copper rolled or drawn, and the remaining arm, on account of the difficulty alluded to, has been formed of brass or other material cast in the desired form.

The object of the present invention is to supply a commutator-bar of pure copper in the described typical form, and by so doing to avoid the disadvantages, both mechanical and electrical, which are involved in uniting two pieces of metal or in using other substances than unalloyed copper for the purpose of forming a commutator-bar.

In the accompanying drawings, illustrative 40 of my invention, Figure 1 is a perspective view of my improved commutator-bar. Fig. 2 is a side view of the same in duplicate, showing the position of the same in a commutator. Fig. 3 is an end view of three such bars in position in a commutator.

In the views the numeral 1 denotes the commutator-bar. The form of this bar admits of considerable variation. It is essential, however, that the bar should have a main arm, 2, which is rubbed by the brushes of the dynamo, and a secondary arm, 3, which serves to con-

nect arm 2 with the appropriate coils, bars, or segments of the rotary armature of the machine to which the commutator is applied. This bar is usually wedge-shaped in cross-section and provided with terminal projections 4 and 5, by means of which it may be clamped in its appropriate position about the armature-shaft, as seen in Fig. 2.

The method or process which I adopt for the manufacture of my improved commutator-bar above described is the ordinary process of drop-forging, and proceeds in the following manner: A cylindrical rod of copper, being cut to the requisite length, is heated to a malleable state, and while in that condition is subjected to the action of successive pairs of dies in a drop-press. By the first pair of dies the so-called operation of "breaking down" and "drawing" the rod is completed. In a second pair of dies the rod is bent and the arms 2 and 3 receive their relative direction. In a third pair of dies the bent copper strip while still hot is subjected to the so-called operation of "striking up," which produces in a rough and ragged state the designed or specified form. The bar is then treated with acid for the purpose of removing oxide. When cold, the product is trimmed in the usual manner. By this means I supply a commutator of pure copper in the typical form above described, or in any desired modification of that form, and at the same time avoid the disadvantages, both mechanical and electrical, which are involved in using two pieces of metal or any other metal than unalloyed copper in a commutator-bar.

Still another advantage possessed by this commutator-bar lies in this, that, being formed from a single copper rod by the process of drop-forging, it has the grain or fiber of the material always parallel to the axis of the commutator-bar, no matter in what shape the same may be bent. This also is an important point, as heightening the conductivity and durability of the article.

In the preferred form of my commutator-bar the outstanding arm has a projection or lug, 6, by which it may be connected conveniently to the coils of the armature.

It is one of the great advantages of this commutator-bar as made by my process of drop-forging that it may be made of any desired and

convenient shape, however complex, and still be of but one piece of metal, homogeneous in molecular structure throughout, and of that great density which is produced by the process of drop-forging, and which is such a desirable quality in a commutator-bar, as affording a high degree of conductivity.

I claim—

1. As an article of manufacture, a full-sized commutator-bar for dynamo-electric machines which has two arms whose longitudinal axes form an angle one with the other, and which is composed throughout of one single piece of unalloyed copper of an almost perfectly homogeneous molecular structure, the fiber or grain of the copper being so arranged as to be everywhere parallel with the axis of the arm and of the greatest possible density, substantially as and for the purpose described.
2. As an article of manufacture, a full-sized commutator-bar for dynamo-electric machines,

which bar as to its shape has two arms whose axes make an angle one with the other, one of which arms has suitable projections at its extremities, by which it may be clamped to the armature-shaft, while the other arm has at its outer extremity a suitable lug or projection, by which it may be connected to the armature-coils, and which bar as to its structure consists of one single piece of unalloyed copper almost perfectly homogeneous throughout, the fiber or grain of the copper being so arranged as to be everywhere parallel with the axis of the arm and of the greatest possible density, substantially as and for the purpose described. 35

In testimony whereof I have hereunto set my name in the presence of two witnesses.

CHARLES E. BILLINGS.

Witnesses:

FRED. C. BILLINGS,  
WILLARD EDDY.